

## UNITED STATES PATENT OFFICE

2,282,163

## TREATMENT OF SILICON-IRON ALLOYS

Stephen L. Burgwin, Wilkinsburg, Pa., assignor  
to Westinghouse Electric & Manufacturing  
Company, East Pittsburgh, Pa., a corporation  
of Pennsylvania

No Drawing. Application February 18, 1941,  
Serial No. 379,481

6 Claims. (Cl. 148—4)

This invention relates generally to the heat treatment of silicon-iron alloys to reduce magnetostriction.

Silicon-iron alloys containing up to 6% of silicon have been utilized for a number of years as the magnetic material in electrical apparatus and particularly as a core member of transformers. Many processes and methods have been employed for heat treating the silicon-iron alloys and fabricating them into strip form suitable for use as the magnetic cores of electrical apparatus. The known processes and methods have for their objective the development of the magnetic characteristics of the alloy by reducing the impurities in the alloy, relieving working strains and/or imparting a preferred orientation to the grain structure of the alloy. The silicon-iron alloys now commercially produced in strip form have excellent magnetic characteristics.

In a number of commercial installations of electrical apparatus, such as large power transformers which utilize the now commercially produced silicon-iron alloy in strip form as the magnetic core member, it has been found that undesirable and objectionable noise is developed when the transformer is energized. The noise developed in a transformer can be traced directly to the magnetostriction of the silicon-iron alloy strips utilized as the core member of the transformer. The magnetostriction of magnetic material is recognized as being the expansion and contraction of the magnetic material when subjected to a magnetizing force. For the purpose of this invention, the kind of magnetostriction of particular interest and the quantity measured is

$$\frac{\Delta L}{L}$$

or the change in length per unit length in the direction of magnetization under the magnetizing force applied.

An object of this invention is to provide for reducing the magnetostriction of silicon-iron alloys which have been fabricated into strip form and treated to develop the magnetic characteristics of the alloy.

A more specific object of this invention is to subject silicon-iron alloys which have been fabricated into strip form and treated to develop the magnetic characteristics of the alloys to a heat treatment suitable for placing the alloys under tension to effectively reduce the magnetostriction of the alloy strip.

Other objects of this invention will become apparent from the following description and the appended claims.

The silicon-iron alloys containing up to 6% silicon are well-known and the processes for de-

veloping the magnetic characteristics of such alloys have been commercially practiced in the past. For example, silicon-iron alloys containing up to about 4½% of silicon are commercially produced in strip form by subjecting them to different heat treatments including the step of cold rolling them to the final stages and then subjecting the resulting strip to an anneal at a temperature of 900° C. or higher to develop the magnetic characteristics of the alloy. Silicon-iron alloys containing higher contents of silicon up to about 6% are not being commercially produced by cold rolling processes, since the higher silicon content renders them somewhat brittle and it has, therefore, become customary to hot work such alloys to the final stages after which a final anneal is employed for relieving working strains. Other methods are well-known and practiced for developing the magnetic characteristics of the silicon-iron alloys containing up to 6% of silicon.

In order to reduce the magnetostriction of the commercially produced silicon-iron alloys containing up to 6% of silicon, in accordance with this invention the commercially produced alloy strips are subjected to a further heat treatment for permanently placing the alloyed components of the strip under tension to effectively reduce the magnetostriction of the commercially produced alloys. The heat treatment of this invention consists in heating the commercially produced alloy strip at a preferred temperature between 700° C. and 1200° C. in the presence of a component which is capable of reacting with the silicon-iron alloy to form a thin adherent film on the surfaces of the strip, the thin film having a linear thermal coefficient of expansion less than the linear thermal coefficient of expansion of the silicon-iron alloys so that in the cooled state the adhering film is present in compression while the silicon-iron alloy is maintained under tension. Many reagents may be employed in forming the adhering film on the silicon-iron alloy strip, it being essential, however, that the reagent be selected to produce a resulting film having a linear thermal coefficient of expansion of less than the coefficient of expansion of the silicon-iron strip on which it is formed.

In a preferred method embodying the teachings of this invention, the treated alloy strip is subjected to a heat treatment at a temperature between 700° C. and 1200° C. in an oxidizing atmosphere, such as air, moist air or carbon dioxide atmosphere or a combination thereof for a period of time of not more than 8 minutes, the oxidizing atmosphere reacting with the alloy to form a thin film of oxides which adhere to the alloy strip. The oxide film usually contains silicates. Any suitable furnace may be employed for heating the strips to the desired temperature as they are

pulled or passed through the heating zone. In all cases where the treated strip is given the further heat treatment in the oxidizing atmosphere, it is desired to maintain the period of time of the heat treatment at less than that time which will cause flaking of the oxide when the strip is cooled.

In a modification of the method described hereinbefore, tension is applied to the strip during the heat treatment for the purpose of insuring that the alloying components will be so strained that as the strip is cooled, the film of oxides formed on the strip during the heat treatment will retain the alloying components under tension even after the external tension is removed. In applying tension during the heat treatment, it is desired, however, to maintain the tension below the elastic limit of the alloy strip, it being found that tensions of the order of 500 to 2000 lbs. per square inch during the heating cycle is sufficient for cooperating with the oxide film for effectively reducing the magnetostriction of the alloy strip.

It is not known exactly what change takes place in the components or structure of the alloy when the adhering film is formed thereon and the strip is cooled. The results obtained, however, illustrate quite definitely that the combination of the thin film under compression with the silicon-iron alloy under tension effectively reduces the magnetostriction of the commercially produced silicon-iron strip.

In determining the effect of the thin films formed on the commercially produced strips, different methods have been developed for measuring the magnetostriction of the alloy strips. The results obtained by the different methods are quite close and for this reason, it is believed to be unnecessary to describe the different methods of measuring the magnetostriction of the alloy strip when treated in accordance with this invention. Two methods for measuring the magnetostriction are, however, described in my co-pending application, Serial No. 385,759, filed March 28, 1941, the methods described therein being suitable for measuring the magnetostriction of the strips treated by the method of this invention.

In order to illustrate the improvement in the magnetostriction of commercially produced strips when subjected to the treatment described, the following table may be referred to as giving the magnetostriction values, that is, change in length per length at a given magnetization of 4½% silicon-iron alloy strips after the commercial mill anneal and after it has been given the oxidizing treatment for forming the thin adhering films thereon in accordance with this invention.

| Number | Treatment |      | Magnetostriction $\frac{\Delta L}{L} \times 10^8$ |         |             |         |
|--------|-----------|------|---------------------------------------------------|---------|-------------|---------|
|        |           |      | B=10000                                           |         | B=14000     |         |
|        | Temp.     | Time | Mill anneal                                       | Treated | Mill anneal | Treated |
| 24G    | ° C.      | Min. |                                                   |         |             |         |
| 24G    | 825       | 4    | 120                                               | 82      | 308         | 194     |
| 26E    | 925       | 4    | 190                                               | 32      | 442         | 140     |
| 27E    | 1,025     | 1    | 170                                               | 12      | 400         | 162     |
| 27C    | 1,025     | 2    | 126                                               | 12      | 336         | 188     |
| 28E    | 1,025     | 4    | 132                                               | 16      | 370         | 188     |
| 28C    | 1,025     | 8    | 126                                               | -4      | 388         | 170     |
| 29E    | 1,100     | 1    | 178                                               | 18      | 426         | 168     |
| 29C    | 1,100     | 2    | 210                                               | 0       | 522         | 168     |
| 31E    | 1,100     | 4    | 138                                               | -8      | 350         | 102     |
| 31C    | 1,100     | 8    | 138                                               | -8      | 340         | 164     |

The heat treatment given each of the samples in an atmosphere of air is indicated in the above table. In all cases there is a definite improvement in the magnetostriction values obtained after the commercially produced strip has been treated in accordance with this invention. From the results given, it is evident that a preferred treatment is to oxidize the commercially produced strips at a temperature between 925° C. and 1100° C. for a length of time ranging between one and four minutes.

The films formed by the oxidizing treatment are of the order of  $2 \times 10^{-5}$  inches thick. The films formed have a definite effect in placing the silicon-iron alloy under tension and the stresses set up by such films have been measured by measuring the bending of the strip when the film is etched first from one surface and then from the other. This has been accomplished by electrolytic etching the film from the strip with a 10% solution of sulphuric acid, measuring the bending of the strip and then calculating the tensile stress based on the bending of the strip. Tensions of the order of 1200 lbs. per square inch have been found in strips treated in accordance with this invention.

In another embodiment of this invention, sodium silicate was employed for applying a film during the heat treatment for effectively reducing the magnetostriction of the commercially produced alloys. In employing the sodium silicate, the commercially produced alloy strip is coated with a thin film of sodium silicate solution and then dried at about 200° C., after which the coated strip is subjected to the heat treatment at a temperature between 875° C. and 1000° C. in air for a period of time of about two minutes. When cooled, it is found that a very adherent film is formed on the treated strip and when the magnetostriction of the strip is measured, it is found that a definite improvement in the magnetostriction is obtained. In the following table, there is given the average magnetostriction values obtained on a number of commercially produced 4½% silicon-iron alloy strips before and after the sodium-silicate treatment described.

| Test number | Average magnetostriction $\frac{\Delta L}{L} \times 10^8$ |         |             |         |
|-------------|-----------------------------------------------------------|---------|-------------|---------|
|             | B=10000                                                   |         | B=14000     |         |
|             | Mill anneal                                               | Treated | Mill anneal | Treated |
| 58          |                                                           | 118     | -2          | 284     |
| 59          |                                                           | 50      | 11          | 169     |
| 60          |                                                           | 98      | 28          | 219     |
| 61          |                                                           | 160     | -8          | 332     |

Each of tests 58, 59 and 60 is the average of a number of tests on strips of the same composition which were subjected to the heat treatment at 900° C. for two minutes in air while strips upon which the results for test 61 are based were subjected to a temperature of 1000° C. for two minutes in air. For all cases, a definite improvement in the magnetostriction at 10,000 gauss is obtained, the improvement at 14,000 gauss not being so marked.

The adhering films on the alloy strip definitely improve the magnetostriction. The formation of the adhering films can also be controlled by applying a superficial film to the strip in the form of a carbonate, sulphate or silicate solution. The

coating formed of the solution will evolve oxygen during the heat treatment to effect an adjustment in the oxygen content of the annealing atmosphere and thereby control the formation of the adhering oxide film on the alloy strip. Strontium carbonate can be effectively employed in this manner for controlling the formation of the adhering oxide film on the strip. Further, by employing the superficial films formed from the solutions of carbonates, sulphates or silicates, it is possible to utilize hydrogen or nitrogen or combinations thereof as the annealing atmosphere, the oxygen evolved from the superficial films being sufficient to effect the formation of the adhering oxide films to establish stresses in tension in the alloy strip and reduce the magnetostriction of the strip.

From the results given hereinbefore, it is quite evident that the method of treating the silicon-iron alloy containing up to 6% of silicon which has been fabricated into strip form and treated to develop its magnetic characteristics at a temperature between 700° C. and 1200° C. in the presence of a component capable of reacting with the silicon-iron alloy to form a thin film on the surface of the strip for placing the alloy under tension effectively reduces the magnetostriction of the alloy.

While this invention has been described with reference to particular embodiments thereof, it is, of course, not to be limited thereto except insofar as is necessitated by the prior art and the scope of the appended claims.

I claim as my invention:

1. In the method of reducing magnetostriction in silicon-iron alloy containing up to 6% of silicon and which has been fabricated into strip form and treated to develop its magnetic characteristics, in combination, coating the treated alloy strip with sodium silicate, subjecting the coated strip to a heat treatment at a temperature between 900° C. and 1100° C. in air for a period of time of not more than three minutes to effectively oxidize the strip and form a thin fused adhering film thereon, and cooling the alloy strip with the adhering film of oxidized and fused material thereon, the adhering film having a linear thermal coefficient of expansion less than the linear thermal coefficient of expansion of the silicon-iron alloy to give a strip in which the silicon-iron alloy is under tension and the adhering film is in compression to effectively reduce the magnetostriction of the alloy strip.

2. In the method of reducing magnetostriction in silicon-iron alloy containing up to 6% of silicon and which has been fabricated into strip form and treated to develop its magnetic characteristics, in combination, heating the treated alloy strip to a temperature between 700° C. and 1100° C. in the presence of a reagent capable of reacting with the silicon-iron alloy to form a thin film of oxidized material on the surfaces of the strip while applying tension to the strip, the tension applied being below the elastic limit of the alloy strip, and cooling the alloy strip with the thin film of oxidized material thereon as an adherent part thereof, the reagent being selected to form a thin film of oxidized material having a linear thermal coefficient of expansion less than the linear thermal coefficient of expansion of the silicon-iron alloy to give a strip in which the silicon-iron alloy is under tension and the adhering film of oxidized material is in compression to effectively reduce the magnetostriction of the alloy strip.

3. In the method of reducing magnetostriction in silicon-iron alloy containing up to 6% of silicon and which has been fabricated into strip form and treated to develop its magnetic characteristics, in combination, heating the treated alloy strip at a temperature between 925° C. and 1100° C. in an oxidizing atmosphere for a period of time of not more than five minutes to form a thin film of oxidized material on the surfaces of

10 the strip while applying tension to the strip, the tension applied being below the elastic limit of the alloy strip, and cooling the oxidized strip to retain the oxidized film as an adherent part thereof, the thin oxidized film having a linear coefficient of expansion less than the linear coefficient of expansion of the silicon-iron alloy to give a strip in which the adhering oxidized film maintains the silicon-iron alloy under tension to effectively reduce the magnetostriction of the 20 alloy strip.

4. In the method of reducing magnetostriction in silicon-iron alloy containing up to 6% of silicon, and which has been fabricated into strip form and treated to develop its magnetic characteristics,

25 in combination, heating the treated alloy strip to a temperature between 825° C. and 1100° C. in the presence of a reagent capable of reacting with the silicon-iron alloy to form a film of oxidized material containing silicates having a thickness of about  $2 \times 10^{-5}$  inches thick on the surfaces of the strip while applying tension to the strip, the tension applied being below the elastic limit of the alloy strip, and cooling the alloy strip with the film of oxidized material containing silicates thereon as an adherent part thereof, the film of oxidized material containing the silicates having a linear thermal coefficient of expansion less than the linear coefficient of expansion of the silicon iron alloy to give a strip 30 in which the silicon-iron alloy is under tension and the adhering film of oxidized material containing silicates is in compression to effectively reduce the magnetostriction of the alloy strip.

5. In the method of reducing magnetostriction in silicon-iron alloy containing up to 6% of silicon and which has been fabricated into strip form and treated to develop its magnetic characteristics, in combination, heating the treated alloy strip to a temperature between 825° C. and

50 1100° C. in the presence of a reagent capable of reacting with the silicon-iron alloy to form a thin film of oxidized material on the surfaces of the strip while applying tension to the strip, the tension applied being between 500 and 2000 pounds per square inch and maintained below the elastic limit of the alloy strip, and cooling the alloy strip with the film of oxidized material thereon as an adherent part thereof, the thin film of oxidized material having a linear coefficient of expansion less than the linear coefficient of expansion of the silicon-iron alloy, the tension applied during the heating so effecting the straining of the alloying components of the silicon-iron strip that the adherent film of oxidized material having the lower coefficient of expansion maintains the silicon-iron alloy under tension when the strip is cooled to effectively reduce the magnetostriction of the alloy strip.

6. In the method of reducing magnetostriction, in silicon-iron alloy containing up to 6% of silicon and which has been fabricated into strip form and treated to develop its magnetic characteristics, in combination, coating the treated alloy strip with sodium silicate, subjecting the

coated strip to a heat treatment at a temperature between 900° C. and 1100° C. in air for a period of time of not more than three minutes to effectively oxidize the strip and form a thin fused adhering film thereon while applying tension to the strip, the tension applied being between 500 and 2000 pounds per square inch and maintained below the elastic limit of the strip, and cooling the alloy strip with the adhering film of oxidized

and fused material thereon, the adhering film having a linear thermal coefficient of expansion less than the linear thermal coefficient of expansion of the silicon-iron alloy to give a strip in which the silicon-iron alloy is under tension and the adhering film is in compression to effectively reduce the magnetostriction of the alloy strip.

STEPHEN L. BURGWIN.